

## 1

3,239,463

## LUBRICATING OIL COMPOSITION

Edwin C. Knowles, Poughkeepsie, N.Y., and Edward L. Kay, Akron, Ohio, assignors to Texaco Inc., New York, N.Y., a corporation of Delaware  
No Drawing. Filed Mar. 24, 1965, Ser. No. 442,472  
6 Claims. (Cl. 252—33.6)

This application is a continuation-in-part of now abandoned application S.N. 83,182.

This invention relates to a lubricating oil composition characterized by having outstanding load-carrying properties. More specifically, the invention relates to a lubricating oil containing a tertiary alkyl primary amine salt of a tetra-covalent boron acid.

Lubricating oil compositions containing certain organoboron compounds have been formulated heretofore. Amine salts of acid compounds of boric acid and of boro-diol complexes have been employed in lubricating oils to improve resistance to sludge-formation and to improve anti-corrosion properties, see U.S. Patent Nos. 2,497,521 and 2,568,472. Borate esters have also been employed in lubricating oils but their use has been seriously hindered by their hydrolytic instability.

The present invention is concerned with lubricating oil compositions containing tertiary alkyl primary amine salts of tetra-covalent boron "acids" known as chelate-type salts which are represented by the following general formulae:



and



wherein R is a monovalent tertiary aliphatic hydrocarbyl radical having from 5 to 24 carbon atoms, R' is a divalent aryl or alkaryl radical having 6 to 24 carbon atoms and R'' is a divalent aryl or alkaryl radical having 6 to 24 carbon atoms or an aliphatic hydrocarbyl radical having 2 to 4 carbon atoms. The acid-amine salt is present in the lubricating oil in a concentration range from above 0.5 to 5.0 weight percent an amount effective to impart load-carrying properties.

The amine salts for the present invention are prepared by the reaction of boric acid with a polyhydroxy compound or hydroxy carboxylic acid to form the tetra-covalent boron compound which is thereafter reacted with a tertiary aliphatic primary amine. The reaction mixture is diluted with a solvent such as toluene and heated to reflux temperature at normal atmospheric pressure. The solvents are then removed preferably by azeotropic distillation and the amine salt recovered.

The amines employed in the formation of the salts of the chelated tetra-covalent boron "acid" are represented by the formula:



wherein R is a monovalent tertiary aliphatic hydrocarbyl radical having 5 to 24 carbon atoms. Preferably R represents a tertiary aliphatic hydrocarbyl radical having from 11 to 22 carbon atoms. Examples of effective tertiary aliphatic primary amines include t-octylamine, t-dodecylamine, and mixtures of primary aliphatic amines such as commercially available mixtures of t-alkyl primary amines. A commercial mixture of monovalent tertiary aliphatic hydrocarbyl amines having 11 to 14 carbon

## 2

atoms in the aliphatic chain is marketed under the name of Primene 81-R by Rohm and Haas. Another mixture of monovalent tertiary aliphatic hydrocarbyl amines having 18 to 22 carbon atoms in the aliphatic chain is marketed under the name of Primene JM-T by Rohm and Haas.

The chelated tetra-covalent boron "acid" employed in the formation of the present invention are transitory compounds and as such do not exist in the isolated state. They do, however, form stable salts. The "acids" are formed by reacting boric acid with a polyhydroxy compound or hydroxy carboxylic acid which may be illustrated by the following general equation:



wherein R' is a divalent aryl or alkaryl radical having from 6 to 24 carbon atoms.

20 The chelated tetra-covalent boron "acids" employed in the formation of the amine salts of the present invention can be represented by the following formulae:



and



wherein R' is a divalent aryl or alkaryl radical having 6 to 24 carbon atoms, preferably 6 to 12 carbon atoms, and R'' is a divalent aryl or alkaryl radical having 6 to 24 carbon atoms or an aliphatic hydrocarbyl radical having 2 to 24 carbon atoms, preferably 4 to 18 carbon atoms. Examples of effective "acids" are boro catecholate acid, alkyl derivatives of boro resorcinate acid, boro salicylate acid, boro alpha hydroxy decanoate acid, boro beta hydroxy decanoate acid, boro glycolate acid, boro propylene glycolate acid, boro tetramethyl ethylene glycolate acid and boro oxalate acid.

45 Upon the formation of the transitory "acids," described above the amine is reacted therewith to obtain the desired amine salt, the reaction for which may be illustrated by the following general equation:



wherein R is a monovalent tertiary aliphatic hydrocarbyl radical having 5 to 24 carbon atoms and R' is a divalent aryl or alkaryl radical having 6 to 24 carbon atoms.

The effective amine salts are illustrated by the following: t-C<sub>11</sub>—C<sub>14</sub> alkyl primary amine boro catecholate, t-C<sub>11</sub>—C<sub>14</sub> alkyl primary amine boro alkylcatecholate, t-C<sub>11</sub>—C<sub>14</sub> alkyl primary amine boro resorcinolate, t-C<sub>11</sub>—C<sub>14</sub> alkyl primary amine boro alkylresorcinolate, t-C<sub>11</sub>—C<sub>14</sub> alkyl primary amine boro salicylate, t-C<sub>11</sub>—C<sub>14</sub> alkyl primary amine boro alkylsalicylate, t-C<sub>11</sub>—C<sub>14</sub> alkyl primary amine boro alpha hydroxy decanoate, t-C<sub>11</sub>—C<sub>14</sub> alkyl primary amine boro alpha hydroxy alkyldecanoate, t-C<sub>11</sub>—C<sub>14</sub> alkyl primary amine boro glycolate, t-C<sub>11</sub>—C<sub>14</sub> alkyl primary amine boro propylene glycolate, t-C<sub>11</sub>—C<sub>14</sub> alkyl primary amine boro tetramethyl ethylene glycolate, t-C<sub>11</sub>—C<sub>14</sub> alkyl primary amine boro oxalate, t-C<sub>18</sub>—C<sub>22</sub> alkyl primary amine boro catecholate, t-C<sub>18</sub>—C<sub>22</sub> alkyl primary amine boro alkylcatecholate, t-C<sub>18</sub>—C<sub>22</sub> alkyl primary amine boro resorcinolate, t-C<sub>18</sub>—C<sub>22</sub> alkyl primary amine boro alkylresorcinolate, t-C<sub>18</sub>—C<sub>22</sub> alkyl primary

amine boro salicylate, t-C<sub>18</sub>-C<sub>22</sub> alkyl primary amine boro alkylsalicylate, t-C<sub>18</sub>-C<sub>22</sub> alkyl primary amine boro alpha hydroxy decanoate, t-C<sub>18</sub>-C<sub>22</sub> alkyl primary amine boro alpha hydroxy alkyldeconate, t-C<sub>18</sub>-C<sub>22</sub> alkyl primary amine boro glycolate, t-C<sub>18</sub>-C<sub>22</sub> alkyl primary amine boro propylene glycolate, t-C<sub>18</sub>-C<sub>22</sub> alkyl primary amine boro tetramethyl ethylene glycolate, t-C<sub>18</sub>-C<sub>22</sub> alkyl primary amine boro oxalate, t-octyl amine boro catecholate, t-octyl amine boro alkylcatecholate, t-octyl amine boro resorcinolate, t-octyl amine boro salicylate, t-octyl amine boro alkylsalicylate, t-octyl amine boro alpha hydroxy decanoate, t-octyl amine boro alpha hydroxy alkyl decanoate, t-octyl amine boro glycolate, t-octyl amine boro propylene glycolate, t-octyl amine boro tetramethyl ethylene glycolate, and t-octyl amine boro oxalate.

The concentration of the tertiary alkyl primary amine salt of a tetra-covalent boron acid of the invention in a lubricating oil composition is critical. Generally, a concentration ranging from above 0.5 percent by weight to 5.0 percent by weight is essential to impart load-carrying properties to a lubricating oil composition. The preferred concentration range for the additive is from about 0.6 to 2.0 weight percent.

The preparation of specific acid amine salts of tetra-covalent boron "acids" useful in a lubricating oil composition is illustrated in the following examples:

#### EXAMPLE I.—PREPARATION OF CHELATE AMINE BORO SALT OF SALICYLIC ACID

123.6 grams, 2.0 mols of boric acid, 552 grams 4.0 mols, salicylic acid and 500 mls. of benzene were refluxed and the water of the reaction removed by azeotropic distillation. Thereafter 400 grams, 2.0 mols of a mixture of t-alkyl primary amine wherein the t-alkyl radical contains 11 to 14 carbon atoms was added to the reaction mixture. The pot temperature rose from 75° C. to 85° C. After stripping solvents to a pot temperature of 150° C., 944 grams of clear viscous t-C<sub>11</sub>-C<sub>14</sub> primary amine boro salicylate liquid were isolated and at ambient temperature the reaction product solidified.

#### EXAMPLE II.—PREPARATION OF CHELATE AMINE BORO SALT OF ALPHA-HYDROXY DECANOIC ACID

61.8 grams, 1.0 mol of boric acid, 200 mls. of toluene and 376 grams, 2.0 mols, of alpha hydroxy decanoic acid were refluxed and 46 mls. of water were removed by azeotropic distillation. The toluene was stripped at a pot temperature of 195° C. Upon the addition of 195 grams, 1.0 mols of a mixture of t-alkyl primary amines wherein the t-alkyl groups contained 11 to 14 carbon atoms mixture, the pot temperature rose from 50° C. to 92° C. 350 mls. of pentane were added to the reaction mixture and the solution was filtered. Pentane was removed by heating the product and 558 grams of clear amber t-C<sub>11</sub>-C<sub>14</sub> primary amine boro alpha hydroxy decanoate liquid were isolated.

#### EXAMPLE III.—PREPARATION OF CHELATE AMINE BORO SALT OF CATECHOL

61.8 grams, 1.0 mol of boric acid, 220 grams, 2.0 mols of catechol and 200 mls. of toluene were refluxed and 51 mols of water were isolated by azeotropic distillation. Solvents were stripped to a pot temperature of 170° C. Upon cooling to room temperature a solid separated. 195 grams, 0.1 mol of a mixture of t-alkyl primary amine wherein the t-alkyl groups contained 11 to 14 carbon atoms mixture were added and the pot temperature rose from 60° C. to 70° C. A water bath was then used to cool the mixture. Some solids were still present in the reaction mixture and thereafter 500 mls. of pentane were added. The mixture was filtered and stripped of pentane. 391 grams of dark amber t-alkyl C<sub>11</sub>-C<sub>14</sub> amine boro catecholate liquid were isolated.

The lubricating oils of this invention are prepared

from hydrocarbon synthetic lubricating oil bases. The hydrocarbon oils found to be useful for this invention include oils having a viscosity in the range required for lubricating fluids and in particular hydrocarbon mineral oils which include paraffin base, naphthene base, mixed paraffin-naphthene base and mineral oils of the residual or distillate type. The hydrocarbon lubricating base generally has been subjected to solvent refining to improve its oxidation and thermal stability and viscosity-temperature properties as well as solvent dewaxing to remove waxy components and to improve the pour properties of the oil. Broadly speaking, hydrocarbon lubricating oils having an SUS viscosity at 100° F. of between 50 to 2500 are used in the formulation of the improved lubricants of this invention.

The mineral lubricating oils to which the amine salts of this invention are added usually contain other additives designed to impart desirable properties thereto. For example, viscosity index improvers such as the polymethacrylates having a molecular weight ranging from 500 to 25,000 are usually included therein. The VI improver normally used is a polymethacrylate having the following recurring structural unit:



wherein R is an aliphatic radical ranging from butyl to stearyl and n is an integer of more than 1.

The use of various metal base organic type additives has been found effective and are generally incorporated in the lubricating oils of this invention, particularly those oils used in high speed, spark ignition and diesel engines to reduce ring sticking, minimize lacquer formation and carbon deposits.

The hydrocarbon lubricating oils of this invention may also contain other additives such as metal sulfonates to afford additional detergent-dispersant properties, metal dialkyl dithiophosphates to afford additional corrosion and oxidation resistance, and anti-foam agents such as silicone polymers in the amount of about 5 to 200 parts per million, etc.

The esters which constituted the synthetic lubricant composition of this invention are broadly described as esters of hydrocarbyl carboxylic acids. They are high molecular weight materials of lubricating oil characteristics derived from alcohols which are usually aliphatic alcohols containing 1 or more hydroxyl radicals and monocarboxylic acids which are usually aliphatic carboxylic acids containing 1 or more carboxylic acid radicals.

Widely used synthetic ester lubricants are aliphatic diesters of aliphatic dicarboxylic acids containing 6 to 12 carbon atoms. From the standpoint of cost and availability, the preferred dibasic acids are adipic acid, sebacic acid and azelaic acid. The aliphatic alcohols used to form the diesters usually contain at least 4 carbon atoms and up to 20 or more carbon atoms. C<sub>6</sub> to C<sub>18</sub> alcohols are most commonly used. Ether alcohols such as Cello-solve and Carbitol may also be used in the formation of the aliphatic diesters of organic dicarboxylic acids used as the lubricating base in the compositions of this invention. Alcohols containing 2 or more hydroxyl radicals and no hydrogen substituted on the beta carbon atom such as trimethylol propane and pentaerythritol have proven particularly effective in formulating stable high temperature ester lubricants.

Examples of alkyl esters of aliphatic carboxylic acids are the following: di-isoctyl azelate, di-2-ethylhexyl sebacate, di-2-ethylhexyl azelate, di-2-ethylhexyl adipate, di-2-ethylhexyl alkenyl succinate, di-2-ethoxyethyl sebacate, di-2-(2'-methoxy-ethoxy) ethyl sebacate, di-2-(2'-ethylbutoxy) ethyl sebacate, di-2-butoxyethyl azelate, di-2-(2'-butoxy-

ethoxy) ethyl alkenyl-succinate, pentaerythritol tetra-caproate and trimethylol propane tri-isooctanoate.

In addition to such esters, polyester lubricants formed by a reaction of an aliphatic dicarboxylic acid, a di-hydroxy compound and a monofunctional compound, which is either an aliphatic monohydroxy alcohol or an aliphatic monocarboxylic acid, in specified mol ratios are also employed as the synthetic lubricating base in the compositions of this invention; polyesters of this type are described in U.S. 2,628,974 on Polyester Synthetic Lubricants, which issued to R. T. Sanderson on February 17, 1953. Polyesters formed by reaction of a mixture containing specified amounts of 2-ethyl-1,3-hexanediol, sebacic acid, and 2-ethylhexanol and by reaction of a mixture containing adipic acid, diethylene glycol and 2-ethylhexanoic acid illustrate this class of synthetic polyester lubricating bases.

The sulfur analogs of the above-described esters are also used in the formulation of the lubricating compositions of this invention. Dithioesters are exemplified by di-2-ethylhexyl thiosebacate, di-n-octyl thiodipate and the dilaurate of 1,5-pentanedithiol; sulfur analogs of polyesters are exemplified by the reaction product of adipic acid, thio glycol and 2-ethylhexyl mercaptan.

Alkyl-substituted phenols are usually incorporated in the lubricants of the invention as anti-oxidants. The preferred and most commonly used alkyl phenol anti-oxidants is 2,6-di-tertiary octylphenol; 2,6-di-tertiary amyl-4-methylphenol; and 2,6-di-isopropyl-4-methylphenol. Hindered phenols of this type are employed in concentrations between 0.1 and 1.0 weight percent.

Although hindered phenol type anti-oxidants are the most widely used anti-oxidants in the lubricant compositions of the invention, aryl-substituted amine anti-oxidants such as phenylnaphthylamine, phenylene diamine, and diphenylamine are also used in lubricants in conjunction with the extreme pressure additive of the invention. The amine anti-oxidants are employed in the same concentrations as the hindered phenol anti-oxidant.

Organic silicones are normally incorporated in the lubricants of the invention to impart thereto anti-foam properties. The silicones are usually of the dialkyl or mixed alkyl-aryl silicone type. Dimethyl silicone is normally employed as the anti-foam agent. The silicone is incorporated in the lubricant by means of a kerosene concentrate containing 5 to 15 weight percent silicone. A very satisfactory anti-foam agent is a kerosene concentrate 10 weight percent dimethyl silicone. The kerosene concentrate is employed in an amount sufficient to provide a silicone polymer concentration of from 50 to 250 parts per million based on the total lubricant composition.

To demonstrate the excellent improvement in the load-carrying ability of lubricating oil containing the amine salts of the present invention, high speed gear scuff test was used. This test is called the I.A.E. Gear Test and is intended for the evaluation of the load-carrying ability of the scuff limited load-carrying ability of those lubricants used in reduction and accessory drives of turbo-jet and turbo-prop engines. The I.A.E. Gear Test is one of the requirements of the British specification D.E.R.D. 2,487 "Lubricating Oil, Aircraft Turbine Engine, Synthetic Type." The I.A.E. Gear Test is also designed to evaluate the scuff limited, load-carrying ability of aircraft gear hydrocarbon lubricants.

The results of the I.A.E. Gear Test on lubricating oil compositions of the present invention are set forth in the following tables:

Table 1.—I.A.E. gear test

| Oil:                                                                                     | 70 | Tooth load, lbs.<br>20 at 6000 r.p.m. |
|------------------------------------------------------------------------------------------|----|---------------------------------------|
| Base oil B                                                                               |    |                                       |
| Base oil B plus 1.0 wt. percent<br>t-C <sub>11</sub> -C <sub>14</sub> primary amine boro |    |                                       |
| alpha hydroxy decanoate                                                                  | 75 | 85 at 6000 r.p.m.                     |

Base oil B consisted of a paraffin base crude which has been furfural refined, lightly acid treated, clay contacted and solvent dewaxed and has an SUS viscosity at 100° F. of 150.

5 The criticality in the concentration of the additive as well as the load-carrying properties of a synthetic lubricating oil composition are demonstrated by the results given in Table II. Base oil C, which was employed in these tests, was di-2-ethyl hexylsebacate, a synthetic oil of lubricating viscosity.

Table II.—I.A.E. gear test

| Blend:                                                                                  | 15 | Tooth load—pounds<br>2000 r.p.m. test<br>speed |
|-----------------------------------------------------------------------------------------|----|------------------------------------------------|
| Base oil C                                                                              |    | 50, 60                                         |
| Base oil C plus 0.1% t-C <sub>11</sub> -C <sub>14</sub> primary<br>amine borosalicylate |    | 50                                             |
| Base oil C plus 0.25% t-C <sub>11</sub> -C <sub>14</sub> primary<br>borosalicylate      |    | 60                                             |
| Base oil C plus 0.5% t-C <sub>11</sub> -C <sub>14</sub> primary<br>amine borosalicylate |    | 80                                             |
| Base oil C plus 2.0% t-C <sub>11</sub> -C <sub>14</sub> primary<br>amine borosalicylate |    | 140                                            |

25 The foregoing results show that significant load-carrying properties begin when the concentration of the additive is above 0.5 percent by weight, lesser amounts of the additive producing no improvement in load-carrying properties over those of the base oil itself.

30 In addition to the load-carrying properties, the amine salts of the chelated tetra-covalent boron acids of the invention also impart a high degree of oxidation and corrosion resistance to lubricating oil compositions. Many organo borate compounds do not perform as satisfactory 35 additives for lubricants because of their hydrolytic instability. In this respect, the salts of the present invention have another important advantage, namely that the amine salts of the chelated tetra-covalent boron "acids" are hydrolytically stable in both water and lubricating oils.

40 We claim:

1. A lubricating oil containing above 0.5 to 5 percent by weight of an amine salt of a tetra-covalent boron acid, said amine salt having the formula:



45 50 wherein R is a monovalent tertiary aliphatic hydrocarbyl radical having from 5 to 24 carbon atoms and R'' is selected from the group consisting of divalent aryl and alkaryl radicals having from 6 to 24 carbon atoms.

55 55 2. A lubricating oil as described in claim 1 wherein R is a mixture of monovalent tertiary aliphatic hydrocarbyl radicals having from 11 to 14 carbon atoms.

60 60 3. A lubricating oil as described in claim 1 wherein R is a mixture of monovalent tertiary aliphatic hydrocarbyl radicals having from 18 to 22 carbon atoms.

65 65 4. A lubricating oil composition according to claim 1 in which said amine salt is present in a concentration of from 0.6 to 2.0 weight percent.

5. A lubricating oil as described in claim 1 containing above 0.5 to 5.0 weight percent of an amine salt having the formula:



70 75 wherein R is a mixture of tertiary alkyl groups having from 11 to 14 carbon atoms.

6. A lubricating oil as described in claim 1 containing above 0.5 to 5.0 weight percent of an amine salt having the formula:



wherein R is a mixture of tertiary alkyl groups having from 11 to 14 carbon atoms.

References Cited by the Examiner

UNITED STATES PATENTS

|           |        |          |          |
|-----------|--------|----------|----------|
| 2,497,521 | 2/1950 | Trautman | 252—33.6 |
| 2,568,472 | 9/1951 | Trautman | 252—33.6 |

DANIEL E. WYMAN, Primary Examiner.